

Patented Oct. 15, 1946

2,409,319

# UNITED STATES PATENT OFFICE

2,409,319

## PRODUCTION OF FABRICS FROM ALGINIC MATERIALS

John Bamber Speakman, Far Headingley, Leeds,  
and Norman Henry Chamberlain, Headingley,  
Leeds, England, assignors to Cefoil Limited,  
Maidenhead, England

No Drawing. Application December 20, 1943, Serial No. 515,029. In Great Britain Oct. 1, 1942

6 Claims. (Cl. 8—115.5)

1

This application corresponds to the application of John Bamber Speakman, Norman Henry Chamberlain and Cefoil Limited, Serial No. 13,782/42, which was filed in Great Britain on October 1, 1942.

This invention comprises improvements in or relating to the production of fabrics from alginic materials.

Up to the present it has been found possible to prepare two main types of alginic rayon; (a) the alkali-soluble type, such as calcium alginic, (b) alkali-resistant types such as chromium or beryllium alginates and formaldehyde-treated alginic acid.

The alkali-resistant types have been produced by conversion from alkali-soluble types, and have then been woven or knitted in the usual way.

Alginic rayon is, however, most easily made and processed in the form of calcium alginic and in certain instances it is desired to produce fabrics in part from calcium alginic with a view to the removal of the alginic fibres from the fabric after weaving or knitting, or from lace fabrics as described in United States patent specification Serial No. 450,012. It is inconvenient in a factory to multiply unnecessarily the kinds of yarn which are kept as stock material for purposes of manufacture. Furthermore, alkali-resistant yarns, particularly chromium alginic yarns and beryllium alginic yarns, are brittle and, therefore, are difficult to weave into fabrics.

According to the present invention a process for the production of alkali-resistant fabrics from alginic materials comprises the steps of first producing alginic rayon of alkali soluble type, then manufacturing fabric therefrom and thereafter converting the alkali soluble alginic of the fabric to alkali-resistant alginic material. In this way it is possible to prepare calcium alginic rayon or other alkali soluble alginic rayon as the stock material for all purposes and, when alkali-resistant fabrics are required to effect conversion to the alkali-resistant form after manufacture of the fabric. Thereafter the converted fabric can be laundered by the usual processes and if desired dyed in alkaline baths without detriment.

The conversion to alkali-resistant material may be effected by treatment with basic chromium or beryllium salts, or with formaldehyde.

When the alkali soluble alginic rayon consists of calcium alginic the calcium may be first removed for combination with alginic acid by treatment with acid and thereafter the fabric is treated (a) with basic chromium or beryllium salt, or (b) with formaldehyde, or (c) with both basic chromium or beryllium salts and with formaldehyde.

It will be understood that in the case of treatment with formaldehyde, the treatment may only be applied after the calcium has been removed,

2

but in the case of treatment with basic chromium or beryllium salts removal of calcium is optional.

In general it may be stated that calcium may be completely removed from fabrics made of calcium alginic by treatment with cold, dilute acids, such as hydrochloric acid. Sulphuric acid is not suitable owing to the insolubility of calcium sulphate in water and aqueous solution, unless delustering of the filaments is not undesirable. The precise conditions under which the extraction is carried out will vary according to the nature and properties of the fabric concerned. Thick, heavy, closely-woven fabrics will require a more prolonged extraction treatment than thin, light, or loosely-woven material. The concentration of acid used is commonly 0.5 N, but this is by no means critical, and complete extraction can be brought about, having due regard to time of treatment and quantity of acid used, by any acid solution having a pH value of less than 3.0 and which forms a soluble salt with calcium.

Strong solutions of mineral acids are not suitable, e. g. hydrochloric acid in concentrations greater than 1.0 N since, although they extract the calcium effectively, they have a tendering action on the material processed.

The acid solution may be circulated about or through the fabric, if it be a very dense one, or treatment may be carried out by simply steeping the fabric in one or more changes of the acid solution. In all cases the acid treatment must be followed by thorough washing in water containing no calcium ions, otherwise the fabric will recalcify during the washing process.

The following is an example of the step of removing calcium:

### Example I

Sixty-six grams of dry calcium alginic fabric, free from oil, are steeped in 3000 cc. of 0.5 N hydrochloric acid for 15 minutes at room temperature. The acid is poured off, and the fabric washed for 4 hours in three changes of distilled water, 5000 cc. being used for each change. The ash content of the fabric is reduced from 13.0% to 0.36% by this treatment.

The following are examples of the step of rendering the fabric insoluble:

### Example II

The treatment of this example may be applied either with or without prior removal of calcium as indicated in Example I.

Basic beryllium acetate solution is prepared by dissolving beryllium carbonate in one half of the quantity of acetic acid theoretically required to form the normal acetate, boiling the solution to expel carbon dioxide, and diluting the resulting liquid until it contains 5% (w./v.) of basic beryllium acetate.

Calcium alginate fabric is extracted with hydrochloric acid and washed in the manner already described, and is then, without drying, treated for 15 minutes or upwards at room temperature with the 5% basic beryllium acetate solution using a fabric-liquor ratio of 100:1 followed by further washing and drying. Fabric so treated contains approximately 5% beryllium and is resistant to alkaline solutions from pH 12 downwards.

Alternatively, the calcium alginate may be treated directly with the basic beryllium acetate solution, without prior removal of calcium. In this case it is preferable to dilute the acetate solution to 2% concentration, and treat the fabric with several successive changes of this diluted solution. The take-up of beryllium is slower and less complete in this case, but satisfactory alkali-resistant materials can be prepared by this method.

*Example III*

The following is an example of the treatment of alginate fabric with basic chromium salts. The general lines of treatment are identical with those described above with basic beryllium salts.

Two hundred grams chrome alum are dissolved in 1500 cc. of cold water, and 31.8 g. anhydrous sodium carbonate in 400 cc. cold water. The two solutions are mixed with constant stirring, and when effervescence of carbon dioxide has ceased, the liquid is made up to 2000 cc., to give a stock solution of basic chromium sulphate containing approximately 2 g. chromium per 100 cc.

Fifty grams of alginate fabric are placed in 1200 cc. water, and 300 cc. of the stock basic chromium sulphate solution is run in, with constant stirring. Treatment is allowed to proceed at room temperature for 3½-4 hours, with occasional agitation, after which the material is washed in running water until free from soluble chromium salts, and dried. The resulting material contains 3-4% chromium, calculated on the dry weight of the fabric, and is satisfactorily resistant to alkalis.

The treatment with basic chromium sulphate solution may follow extraction with hydrochloric acid for removal of calcium as already described.

*Example IV*

The following is an example of the treatment of alginate fabric with formaldehyde.

When calcium alginate fabrics are to be treated with formaldehyde for the purpose of rendering them resistant to alkalis, it is always necessary to extract the calcium first by the methods already described.

The extracted and washed fabric is steeped for 30 minutes at room temperature in a solution containing 20% formaldehyde and 5% of ammonium chloride, the pH of the solution being adjusted to approximately 3.5 (working limits, 3.0-4.0; certainly not greater than 4.0). After steeping, the surplus liquid is removed by squeezing, and the fabric at once transferred to an oven at 98° C. for 90 minutes or longer. The material so treated is satisfactorily resistant to alkalis.

*Example V*

The following is an example of the treatment of alginate fabrics with formaldehyde in vapour form.

The calcium alginate fabric is extracted with hydrochloric acid to remove calcium, washed, and

dried. It is then suspended in a chamber heated to approximately 100° C. by a steam jacket or other suitable means. Formaldehyde vapour is obtained by heating para-formaldehyde, either in the main chamber itself, or in a subsidiary compartment so arranged that the vapour evolved passes into the main chamber containing the fabric. In the latter case, the vapours are preferably dried by passing them over trays of anhydrous calcium chloride. Alternatively, calcium chloride, may be placed on shelves or trays in the main chamber.

Material so treated for 1 hour shows an extremely high resistance to alkalis, and its strength is considerably increased, particularly in the wet state.

Since the reaction which proceeds during the treatment of extracted alginate fabrics with formaldehyde consists in the formation of methylene bridges between adjacent hydroxyl groups of the mannuronic acid residue chains, the carboxyl groups of the structure are unaffected, and are therefore available in the formaldehyde-treated material for subsequent combination with basic beryllium or chromium salts. It is therefore clear that any or all of the treatments with basic beryllium or chromium salts already detailed may be applied equally well to material which has already been treated with formaldehyde either in liquid or gaseous form. While such double treatment would not normally be necessary in order to confer adequate alkali-resistance, it might upon occasion be necessary in cases where the utmost resistance to alkaline solutions was required.

The treatments described are equally applicable to knitted and woven fabrics, and to fabrics consisting of calcium alginate in combination with other textile materials such as cotton, wool, viscose or casein fibre.

We claim:

1. A process for the production of alkali-resistant fabrics from alginic materials, comprising the steps of first producing alginate rayon of alkali-soluble type, then manufacturing fabric therefrom and thereafter converting the alkali soluble alginate of the fabric to alkali-resistant alginic material.

2. A process as claimed in claim 1, wherein the conversion to alkali-resistant material is effected by treatment with basic salts of metals selected from the class consisting of chromium and beryllium.

3. A process as claimed in claim 1, wherein conversion to alkali resistant material is effected by treatment with dilute basic beryllium acetate solution.

4. A process as claimed in claim 1, wherein the conversion to alkali-resistant material is effected by treatment with dilute basic chromium sulphate solution.

5. A process for the production of alkali-resistant fabrics from alginic materials, comprising the steps of first producing calcium alginate rayon, then manufacturing fabric therefrom, thereafter removing the calcium from the fabric by treatment with acid and thereupon treating the fabric with formaldehyde.

6. A process as claimed in claim 5, wherein the extraction of calcium from the rayon in the fabric is effected by treatment with hydrochloric acid.

JOHN BAMBER SPEAKMAN.  
NORMAN HENRY CHAMBERLAIN.